

1

3,177,159

HYDROISOMERIZATION OF OLEFIN  
Thomas A. Rodgers, La Porte, and Maxwell Nager, Pasadena, Tex., assignors to Shell Oil Company, New York, N.Y., a corporation of Delaware  
No Drawing. Filed Dec. 27, 1961, Ser. No. 162,601  
3 Claims. (Cl. 252—439)

This invention relates to a process for the catalytic conversion of unbranched or lightly branched hydrocarbons into branched or more highly branched hydrocarbons having the same number of carbon atoms. More particularly, the process relates to the isomerization of normal olefins to isoparaffins having the same number of carbon atoms. The invention more particularly relates to the application of a special catalyst for carrying out the isomerization.

Normal olefins in the gasoline boiling range have a high octane rating, particularly blending octane rating. However, their presence in motor gasoline in recent years has been increasingly undesirable because of their high sensitivity. By sensitivity it is meant the difference in octane rating determined by the Research Method (F-1) and the octane rating determined according to the Motor Method (F-2).

It is known that olefins can be converted to the corresponding saturated hydrocarbons by hydrogenation, usually by a catalytic process employing a catalyst comprising a hydrogenation component on an inert support, such as the conventional cobalt molybdenum on alumina catalyst. However, while the Research octane rating of normal olefins is relatively high, the Research octane rating of the normal paraffin product obtained by simple hydrogenation is often very much lower. Therefore, simple hydrogenation processes have not been looked upon with favor since the refiner can rarely tolerate the loss in Research octane rating.

It has been proposed to hydroisomerize olefins by means of a dual function catalyst comprising a hydrogenation component associated with an acid-acting support. In such a process, normal olefins are converted at an elevated temperature and pressure into isoparaffins. Isoparaffins have a considerably higher octane rating than the corresponding normal paraffins, thus, the hydroisomerization product is not only of the desired degree of saturation, but owing to the increase in isoparaffin content, is of a higher research octane rating than the product obtained by a conventional simple hydrogenation process. Further details of the hydroisomerization of olefins are disclosed and described in copending application Serial No. 39,818, filed June 30, 1960, now Patent No. 3,149,180, by Joost C. Platteeuw and Johannes H. Choufoer.

The mechanism by which normal olefins are converted into isoparaffins in the presence of a dual function catalyst is not fully understood, although the simplest explanation is that the olefins are first isomerized to an isoolefin which is then hydrogenated to the corresponding isoparaffin. That the isomerization reaction proceeds before the hydrogenation reaction is supported by the observation that normal paraffins are substantially unaffected by the catalyst at the conversion conditions.

For the commercial practice of a catalytic hydroisomerization process, the catalyst should be selective and stable, i.e., the catalyst should have the ability to convert

2

the non-highly branched olefins into highly branched paraffins for an extended period of time. It is generally considered that selectivity is a measure of the ability of the catalyst to provide a high ratio of highly branched hydrocarbons to unbranched or lightly branched hydrocarbons whereas stability is a measure of the ability of the catalyst to convert olefins into paraffins.

A hydroisomerization catalyst having a high selectivity is comprised of nickel sulfide on an acid-acting support such as acidic refractory oxides. For example, in the conversion of a normal olefin, e.g., hexene-1, with such a catalyst, the ratio of isoparaffin to normal paraffin in the product is at least 7:1. However, in use, the nickel sulfide catalyst rapidly loses its ability to convert the olefin to paraffins. Therefore, as olefins begin to appear in the product in substantial quantities, it is the practice to increase the conversion temperature to maintain the desired degree of saturation. Ultimately, however, usually after only a few hundred hours operation, a point is reached where the conversion temperature has been raised to the maximum temperature desired for the process and it becomes necessary to interrupt the process and to reactivate or renew the catalyst.

It is an object of this invention to provide an improved process for the hydroisomerization of normal or lightly branched olefins to more highly branched paraffins. It is a particular object of this invention to provide an improved process for the hydroisomerization of olefins by means of a special catalyst which is selective and yet highly stable.

It has now been found that stability of nickel sulfide hydroisomerization catalyst is greatly improved by incorporating a critically small amount of tungsten in the catalyst. Thus, the addition of tungsten to the nickel sulfide catalyst permits the hydroisomerization process to be carried out for a much longer period of time than that which is obtained with the nickel sulfide catalyst without tungsten.

The amount of nickel in the hydroisomerization catalyst can vary within wide limits and generally is in the range of from about 0.5 to about 20% by weight based on the total catalyst. For a particularly active catalyst, the amount of nickel is preferably in the range from about 6 to about 12% by weight based on the total catalyst.

The atomic ratio of nickel to tungsten in the catalyst should be greater than 10:1 and preferably greater than 15:1. With a catalyst containing higher proportion of tungsten, that is at a nickel to tungsten atomic ratio of less than 10:1 the selectivity, although high initially, levels out after a few hours at a level which is about the same as that obtained with a conventional hydrogenation catalyst such as cobalt molybdenum on alumina. On the other hand, to obtain the benefits of the invention to an appreciable degree, the nickel to tungsten ratio should be not more than about 150:1 and preferably no more than about 125:1. A particularly preferred range for the nickel:tungsten atomic ratio is about 20:1 to 80:1.

The tungsten and nickel components of the catalyst are intimately combined with an acid-acting catalyst such as the acid-acting refractory oxides. By an acid-acting catalyst it is meant those which when absorbing butter yellow and still other weaker basic indicators, show a color change of these indicators, indicating the transition to

the acid form. Suitable acid-acting catalyst for the dual function hydroisomerization catalyst of the invention are compounds of silica and alumina such as silica-alumina cracking catalyst, compounds of silica and zirconium dioxide, compounds of boron trioxide and alumina, compounds of boron trioxide and silica, and the like. The catalyst consisting of silica-alumina compounds, in particular those having a silica content of at least 60% by weight and an alumina content of about 1 to 40% by weight are preferred.

The tungsten and nickel can be applied to the acid-acting catalyst, for instance silica-alumina cracking catalyst, by any suitable method known per se. For example, the tungsten and nickel can be applied by impregnating the acid catalyst with a solution of a salt of the corresponding metal, for example, nickel nitrate and silicotungstic acid, which is then followed by drying and calcining.

The tungsten and nickel are converted at least in part to the sulfide form before use in the hydroisomerization process. The catalyst can be sulfided before placement in the reaction vessel or it can be sulfided in situ within the reactor vessel. The sulfiding can be carried out by any manner conventionally known in the art, such as by contacting the catalyst with a mixture of hydrogen sulfide and hydrogen or by contacting the catalyst at a low temperature with a hydrocarbon containing a small amount of decomposable sulfur compound such as about 1-3% by volume carbon disulfide.

The process of the invention is particularly suitable for the conversion of unbranched or lightly branched olefins boiling within the gasoline boiling range into more highly branched paraffins. The process is especially suitable for the conversion of unbranched or lightly branched olefins having from 4 to 8 carbon atoms per molecule into more highly branched paraffinic hydrocarbons. The olefinic starting material can be one or more olefins or can be a mixture of one or more olefins and other hydrocarbons. The olefinic starting material to be converted is generally passed over the dual function catalyst at a liquid hourly space velocity of from about 0.5 to about 20 barrels of liquid hydrocarbons per hour per barrel of catalyst, although lower or higher space velocities may also be used.

The conversion of olefins in the present process is carried out in the presence of hydrogen and at an elevated pressure, preferably at a total pressure not exceeding 1500 pounds per square inch, and in particular at a total pressure from about 150 to about 1500 pounds per square inch. The hydrogen partial pressure may vary within wide limits and is preferably from about 50% to about 95% of the total pressure. Pure hydrogen is not necessarily used, as hydrogen containing gases, such as the hydrogen rich gases from a reforming process, are also suitable.

Conversion of the olefin is carried out at an elevated temperature generally in the range of from 400° to 900° F. and preferably 500° to 750° F.

The following examples further illustrate the process of the invention and its advantages.

#### EXAMPLE I

A series of catalytic compounds comprising silica-alumina, nickel sulfide and tungsten sulfide were prepared in the following manner. A commercially available silica-alumina cracking catalyst containing approximately 25% alumina and 75% silica was employed as the acid-acting support. The silica-alumina, in the form of  $\frac{1}{8}$ " pellets, was impregnated with an aqueous solution of nickel nitrate and silicotungstic acid, the strength of the nickel nitrate solution being selected to provide approximately 6.5% by weight nickel based on the total catalyst. The concentration of the silicotungstic acid solution was varied so as to deposit the desired quantity of tungsten onto the silica-alumina. Total volume of impregnating

solution used was about 0.9 cc. per gram of silica-alumina. The wetted pellets were allowed to stand for approximately 16 to 20 hours, and were then dried with stirring, under a heat lamp. The catalyst was then dried for an additional 3 hours at 266° F. in a vacuum. The dried catalyst was calcined at 482° F. for 20 hours and then calcined for an additional 5 hours at 860° F.

For comparison, another catalyst was prepared in a similar manner, but without the addition of tungsten. This catalyst contained 9.9% nickel, based on the weight of the total catalyst.

Prior to use, the catalysts were sulfided in the reaction vessel, using 3% by volume carbon disulfide in light naphtha. The sulfiding temperature was raised from approximately 270° F. to the desired hydroisomerization temperature at the rate of about 55° F. per hour.

A total of five nickel catalyst composites were prepared. Catalysts "A," "B," "C," and "D" contained 0.25%, 1.0%, 2.5% and 10.0% by weight tungsten, respectively, which provided a nickel to tungsten atomic ratio of 81.5, 20.4, 8.2, and 2.0, respectively. Catalyst "E" contained 9.9% by weight nickel and no tungsten.

The five catalysts were individually employed in the hydroisomerization of a wide boiling range (120-365° F.) hydrocarbon fraction comprising on a volume basis approximately 75% cracked gasoline and 25% straight-run naphtha. Properties of the hydrocarbon fraction are given in Table I.

Table I

## PROPERTIES OF HYDROISOMERIZATION FEED

|                                         |      |
|-----------------------------------------|------|
| API gravity at 60° F.                   | 54.8 |
| Group hydrocarbon type, percent v. FIA: |      |
| Saturates and naphthenes                | 38   |
| Olefins                                 | 36   |
| Aromatics                               | 26   |
| Bromine No.                             | 57   |
| Maleic anhydride value                  | 4.1  |
| Nitrogen, p.p.m.                        | 35   |
| Sulfur, p.p.m.                          | 310  |
| Molecular weight                        | 106  |
| ASTM Dist., ° F.:                       |      |
| IBP                                     | 120  |
| 5%                                      | 154  |
| 10%                                     | 173  |
| 30%                                     | 216  |
| 50%                                     | 254  |
| 70%                                     | 288  |
| 90%                                     | 329  |
| 95%                                     | 350  |
| EP                                      | 365  |

The hydroisomerization reaction was carried out at 750 p.s.i.g., 1.3 LHSV, and 5 H<sub>2</sub>/oil molar ratio. Reactor outlet temperature was raised as necessary up to a limit of 800° F. to maintain a product which was 95% saturated. The ratio of isopentane to normal pentane in the product was determined to indicate selectivity of the particular catalyst for the hydroisomerization reaction.

The addition of tungsten to the nickel catalyst improved stability greatly, as indicated by a run life of about 735 and 1125 hours obtained for catalysts A and B, respectively, compared with a run life of only 650 hours obtained for catalyst E, which contained no tungsten.

After an initial sharp decline, selectivity of the tungsten-containing catalysts remained substantially constant for the remainder of the run period. With catalyst E, which contained no tungsten, selectivity declined gradually throughout most of the run period.

Thus, at the end of 200 hours, when the selectivity had become substantially stabilized, selectivity for catalysts A through E was 6.0, 3.5, 2.3, 2.3, and 6.8, respectively. The selectivity of 2.3 for catalysts C and D was substantially the same as that obtained with a conventional cobalt molybdenum hydrogenation catalyst under the same conditions. Thus, the amount of tungsten add-

ed to the nickel catalyst should be kept relatively low so as to obtain the advantages of the hydroisomerization conversion.

We claim as our invention:

1. A catalyst which comprises nickel and tungsten deposited on an acid-acting support, the atomic ratio of nickel to tungsten being from about 10 to 1 to about 150 to 1, the amount of nickel being from about 0.5 to about 20% by weight, based on the total catalyst, and said nickel and tungsten being in the form of a sulfide.

2. A catalyst which comprises nickel and tungsten deposited on an acid-acting refractory oxide support, the atomic ratio of nickel to tungsten being from about 10 to 1 to about 150 to 1, the amount of nickel being from about 0.5 to about 20% by weight, based on the total catalyst, and said nickel and tungsten being in the form of a sulfide.

3. A catalyst which comprises nickel and tungsten deposited on silica-alumina, the atomic ratio of nickel to

tungsten being from about 10 to 1 to about 150 to 1, the amount of nickel being from about 0.5 to about 20% by weight, based on the total catalyst, and said nickel and tungsten being in the form of a sulfide.

5

References Cited by the Examiner

UNITED STATES PATENTS

|           |       |                |            |
|-----------|-------|----------------|------------|
| 2,554,282 | 5/51  | Voorhies       | 252—439    |
| 2,595,772 | 5/52  | Daussat et al. | 252—439    |
| 2,744,052 | 5/56  | Nozaki         | 208—143    |
| 2,943,127 | 6/60  | Carr           | 260—683.65 |
| 2,982,802 | 5/61  | Folkins et al. | 260—683.65 |
| 3,078,238 | 2/63  | Beuther et al. | 208—143    |
| 3,116,232 | 12/63 | Noger et al.   | 260—683.65 |

10

15

FOREIGN PATENTS

878,035 9/61 Great Britain.

ALPHONSO D. SULLIVAN, Primary Examiner.